

Jan. 28, 1964

M. A. BLUMENFELD ET AL

3,119,754

### ELAPSED TIME INDICATOR

Filed Feb. 10, 1961



FIG. 1.



FIG.2.

*INVENTORS*  
MARTIN A. BLUMENFELD  
LIEN Y. LI  
BY

BY

Henry Knapp  
ATTORNEY

1

3,119,754

ELAPSED TIME INDICATOR

Martin A. Blumenfeld, Somerville, N.J., and Lien Yen Li, Glen Cove, N.Y., assignors to Sperry Rand Corporation, Great Neck, N.Y., a corporation of Delaware  
Filed Feb. 10, 1961, Ser. No. 88,488  
5 Claims. (Cl. 204—52)

The present invention generally relates to elapsed time indicators of the electrolytic cell type and, more particularly, to such an indicator suitable for use over relatively wide temperature ranges.

Elapsed time indicators of the electrolytic cell type are well known in the art as comprising an anode element, a cathode element and an electrolytic solution housed in a sealed container. The cell is energized by causing a constant direct current to flow between the anode and cathode elements during the time interval to be measured. While the current is flowing, metal is transferred at a predetermined rate from the anode to the cathode of the electrolytic cell. The total elapsed time is directly related to the erosion of the anode and can be easily measured by calibrating the length of the anode element.

One of the primary uses of the electrolytic cell is to measure the length of time that electrical equipment has been in operation so that preventative maintenance procedures can be undertaken at proper intervals. For this purpose, the cell is energized concurrently with said equipment. A problem arises, however, when the electrolytic cell is subjected to extreme temperature variations such as are encountered during the flight of present day high altitude aircraft. Temperature changes of such magnitude adversely affect the accuracy of the elapsed time indication and can actually destroy the cell.

It is of course desirable that the plating action on which the elapsed time indication is based be substantially independent of temperature. More particularly, it is necessary that an electrolytic solution be provided which satisfies the following requirements over the entire temperature range of operation such as, for example, from —55° C. to 110° C. The solution must facilitate the sound deposition of metal on the cathode element of the electrolytic cell. Both anode and cathode efficiency should approach 100 percent. Gassing of the solution and anode sludging should be kept to a minimum. Anode erosion must be relatively uniform and in accordance with Faraday's laws. The solution must remain liquid throughout the temperature range.

A cursory consideration of the problem might suggest merely adding conventional antifreeze agents such as alcohol or ethylene glycol to prior art electrolytic solutions to achieve the required low temperature operation. It has been found, however, that when such agents are added to a copper fluoborate electrolytic solution, considerable salting out occurs at the low temperatures. Moreover, the addition of organic agents such as methyl and ethyl alcohol seriously impede plating at high temperatures because of the low boiling points of the additives.

In accordance with the present invention, the aforementioned requirements are met directly by a unique proportioning of the prior art copper fluoborate electrolytic solution constituents. No additives foreign to the original solution are required.

It is the principal object of the present invention to provide an improved electrolyte for an elapsed time indicator of the electrolytic cell type suitable for use over wide variations in temperature.

Another object of the present invention is to provide an improved elapsed time indicator of the electrolytic cell type for use over relatively wide temperature ranges.

2

A further object is to provide an electrolytic solution for electro-depositing copper at a rate which is substantially independent of temperature over a wide range.

These and other objects of the present invention, as will appear from a reading of the following specification, are achieved in a preferred embodiment by the provision of an electrolytic cell comprising a copper anode, a copper cathode and an electrolytic solution housed in a sealed glass envelope. Means are provided for passing a constant current through the anode and cathode elements whereupon metallic copper is eroded from the anode and deposited upon the cathode. The rate of metallic copper transference from the anode to the cathode is maintained substantially independent of temperature over a range from about —55° C. to about 110° C. through the use of an appropriately proportioned copper fluoborate solution.

The copper fluoborate solution consists of copper fluoborate  $\text{Cu}(\text{BF}_4)_2$ , boric acid ( $\text{H}_3\text{BO}_3$ ), fluoboric acid ( $\text{HBF}_4$ ), and distilled water. In accordance with the present invention, the ratio in weight of copper fluoborate to boric acid is substantially 15:1. The relationship between the copper fluoborate, fluoboric acid and water is determined substantially in accordance with the linear expression:

$$y = -940x + 640$$

where  $y$  represents  $\text{Cu}(\text{BF}_4)_2$  as measured in grams per liter of electrolytic solution and  $x$  represents the ratio in weight of  $\text{HBF}_4$  to  $\text{H}_2\text{O}$ .

For a more complete understanding of the present invention, reference should be had to the following specification and to the figures of which:

FIG. 1 is a simplified schematic diagram of an elapsed time indicator of the electrolytic cell type; and

FIG. 2 is a plot of the relationship between the copper fluoborate, fluoboric acid and water constituents of the electrolytic solution as determined in accordance with the present invention.

Referring to FIG. 1, the elapsed time indicator comprises a high silicon glass envelope 1 which is adapted at opposite ends 2 and 3 for the insertion of conductors 4 and 5. Conductors 4 and 5 are sealed to glass envelope 1 by means of a suitable glass-to-metal seal 9 such as Kovar. Conductor 4 supports tubular glass guide 6 which encases high-purity (oxygen-free) copper anode 7. A direct electrical connection is made between conductor 4 and anode 7. Cathode 8 comprises essentially the same high-purity copper as used for anode 7 and is supported adjacent end 3 of tube 1 by conductor 5. A direct electrical connection is made between cathode 8 and conductor 5.

Substantially all of the remaining volume contained within envelope 1 is filled with a copper fluoborate electrolytic solution 11. It is preferred to prevent exposure of conductors 4 and 5 to solution 11 by covering the conductors with glass 10 along those portions which are interior to envelope 1. An expansion chamber or protrusion 12 is provided to allow for the expansion of solution 11 at elevated temperatures. Solution 11 only partially fills chamber 12 leaving an entrapped volume of air 13 which is compressed upon the expansion of solution 11.

The basic operation of the electrolytic cell is well known in the art. Briefly, it involves the passing of an essentially constant D.C. current between conductors 4 and 5. The resulting transference of the metallic copper from anode to cathode proceeds at a uniform rate. A series of fiducial marks 14 which may, for example, be inscribed on the wall of glass envelope 1, marks off the length of anode 7. The marks 14 may be used to measure the remaining length of anode 7 at any time during the

operation of the electrolytic cell. The remaining length of anode 7 is a measure of the amount of anode erosion which, in turn, is proportional to the length of time that the D.C. current has been applied between conductors 4 and 5. Thus, where the application of the D.C. current is commensurate with the time that specified electrical apparatus is energized, the total operational time of said apparatus may be determined by reading the remaining length of anode 7.

In accordance with the present invention, the electrolytic cell of FIG. 1 is adapted for operation over a temperature range from about -55° C. to about 110° C. This is accomplished by proportioning the constituents of copper fluoborate solution 11 in the following manner. The copper fluoborate solution consists of copper fluoborate  $[Cu(BF_4)_2]$ , fluoboric acid ( $HBF_4$ ), distilled water, and boric acid ( $H_3BO_3$ ). The ratio in weight of  $Cu(BF_4)_2$  to  $H_3BO_3$  is about 15:1. The relationship between  $Cu(BF_4)_2$ ,  $HBF_4$  and  $H_2O$  is determined substantially in accordance with the expression  $y = -940x + 640$  where  $y$  represents  $Cu(BF_4)_2$  as measured in grams per liter of electrolytic solution, and  $x$  represents the ratio in weight of  $HBF_4$  to  $H_2O$ . This relationship is represented in graphical form in the plot of FIG. 2.

Referring to FIG. 2 which is a plot of the expression  $y = -940x + 640$ , it has been found that the relationship between the copper fluoborate, fluoboric acid and water must be such as to define points along the straight line. Solutions which may be represented by points lying above the line exhibit too high a specific resistance especially at low temperatures. Solutions represented by points lying below the line tend to "salt out" or freeze or both at the low temperatures. Additionally, the concentration of copper fluoborate in grams per liter of electrolytic solution should be no greater than approximately 430 and no less than approximately 40. A concentration of greater than 430 grams per liter produces a tendency of the solution to "salt out" at low temperatures whereas a concentration less than 40 grams per liter seriously weakens the efficiency of the transference of copper between the anode and cathode elements at all temperatures. However, when the relationship between copper fluoborate, fluoboric acid and water is such as to define points substantially along the straight line of FIG. 2 between the ordinates of 430 and 40 grams per liter, and the ratio of copper fluoborate to boric acid is maintained at about 15:1, a solution is produced which facilitates the efficient operation of the elapsed time indicator of FIG. 1 substantially independent of temperature over the range between -55° C. and 110° C.

A typical fluoborate electrolytic solution, prepared in accordance with the present invention, consists of the following proportions of the constituents,

| Constituent:           | Gm./liter |
|------------------------|-----------|
| $Cu(BF_4)_2$ -----     | 166       |
| $HBF_4$ -----          | 392       |
| Distilled $H_2O$ ----- | 775       |
| $H_3BO_3$ -----        | 11.1      |

In the above example, the ratio of  $Cu(BF_4)_2/H_2O$  is substantially 0.506. These proportions define point P in the plot of FIG. 2.

While the invention has been described in its preferred embodiments, it is understood that the words which have been used are words of description rather than of limitation and that changes within the purview of the appended claims may be made without departing from the true scope and spirit of the invention in its broader aspects.

What is claimed is:

1. An electrolytic solution for use in an elapsed time indicator of the electrolytic cell type having copper anode and cathode elements, said solution comprising copper

fluoborate of a concentration in the range from about 40 to about 430 grams per liter, boric acid, fluoboric acid and water, the ratio in weight of copper fluoborate to boric acid being about 15:1 and the relationship between the copper fluoborate, fluoboric acid and water being determined substantially in accordance with the expression:

$$y = -940x + 640$$

wherein  $y$  represents the weight in grams of said copper fluoborate per liter of electrolytic solution and  $x$  represents the ratio in weight of fluoboric acid to water.

2. An electrolytic cell comprising an anode element, a cathode element, an electrolytic solution, and a sealed container for housing said elements and said solution, said electrolytic solution comprising copper fluoborate of a concentration in the range from about 40 to about 430 grams per liter, boric acid, fluoboric acid and water, the ratio in weight of copper fluoborate to boric acid being about 15:1 and the relationship between the copper fluoborate, fluoboric acid and water being determined substantially in accordance with the expression:

$$y = -940x + 640$$

wherein  $y$  represents the weight in grams of said copper fluoborate per liter of electrolytic solution and  $x$  represents the ratio in weight of fluoboric acid to water.

3. An electrolytic cell comprising a copper anode, a copper cathode, an electrolytic solution, and a sealed glass envelope for containing said anode, said cathode and said solution, said solution comprising copper fluoborate of a concentration in the range from about 40 to about 430 grams per liter, boric acid, fluoboric acid and water, the ratio in weight of copper fluoborate to boric acid being about 15:1 and the relationship between the copper fluoborate, fluoboric acid and water being determined substantially in accordance with the expression:

$$y = -940x + 640$$

wherein  $y$  represents the weight in grams of said copper fluoborate per liter of electrolytic solution and  $x$  represents the ratio in weight of fluoboric acid to water.

4. An electrolytic solution for electrodepositing copper at a rate which is substantially independent of temperature over a range from about -55° C. to about 110° C., said electrolytic solution comprising copper fluoborate of a concentration in the range from about 40 to about 430 grams per liter, boric acid, fluoboric acid and water, the ratio in weight of copper fluoborate to boric acid being about 15:1 and the relationship between the copper fluoborate, fluoboric acid and water being determined substantially in accordance with the expression:

$$y = -940x + 640$$

wherein  $y$  represents the weight in grams of said copper fluoborate per liter of electrolytic solution and  $x$  represents the ratio in weight of fluoboric acid to water.

5. In an elapsed time indicator of the electrolytic cell type having copper anode and cathode elements, an electrolytic solution by weight consisting of about 166 parts of copper fluoborate, about 392 parts of fluoboric acid, about 775 parts of water and about 11 parts of boric acid.

#### References Cited in the file of this patent

#### UNITED STATES PATENTS

- 65 Re. 24,190 Kroko ----- July 31, 1956  
 2,791,473 Mattox ----- May 7, 1957  
 3,029,384 Hart ----- Apr. 10, 1962

#### OTHER REFERENCES

- Handbook of Practical Electroplating, page 154, Macmillan Co., New York, 1959.